

# UNITED STATES PATENT OFFICE.

HYLEMAN ALISON WEBSTER, OF COLUMBIA, TENNESSEE, ASSIGNEE TO JOHN JEFFERSON GRAY, JR., OF ROCKDALE, TENNESSEE.

## PROCESS OF PRODUCING PHOSPHOR-COPPER COMPOUNDS.

1,265,150.

Specification of Letters Patent.

Patented May 7, 1918.

No Drawing.

Application filed December 28, 1916. Serial No. 139,348.

To all whom it may concern:  
Be it known that I, HYLEMAN ALISON WEBSTER, a citizen of the United States, residing at Columbia, in the county of Maury 5 and State of Tennessee, have invented certain new and useful Improvements in Processes of Producing Phosphor-Copper Compounds; and I do hereby declare the following to be a full, clear, and exact description 10 of the invention, such as will enable others skilled in the art to which it appertains to make and use the same.

This invention relates to a continuous process of producing compositions, or compounds 15 of copper and phosphorus, and has for its object to provide a method which will attain these results when using a basic phosphate as a source of phosphorus in a more efficient and less costly manner than has 20 been heretofore proposed.

With this and other objects in view the invention consists in the novel steps and combinations of steps constituting the process all as will be more fully hereinafter disclosed 25 and particularly pointed out in the claims.

In order that the invention may be clearly understood it is said:—It has long been known that compounds, alloys or physical mixtures of copper and phosphorus, could 30 be made by introducing elemental phosphorus into copper. But the cost of this method of procedure has been found to be so high on account of the almost prohibitive 35 cost and limited supply of pure phosphorus, that the employment or use of these highly useful compositions of copper containing phosphids has been greatly curtailed.

According to this invention, on the other 40 hand, I produce compositions containing copper and phosphorus such as copper phosphids, in a blast furnace, in an electric furnace, or in any other suitable furnace by smelting a charge of the character mentioned below. That is to say, selecting a blast furnace as an example only, I may employ a charge consisting substantially of:—silicia  $SiO_2$  1.1 parts to one part  $CaO$ . Phosphorus ascertained by calculation based 45 on the percentage of tricalcium phosphate in the phosphate rock, 1 part to 2 parts of copper; coke in excess, say 1 part to 2 parts

of the charge. More specifically stated a blast furnace charge may be made up as follows:—

|                           |           |
|---------------------------|-----------|
| Tricalcium phosphate rock | 4000 lbs. |
| Quartz                    | 2120 "    |
| Copper                    | 1200 "    |
| Coke                      | 3600 "    |

55

60

In case an electric furnace is used that portion of the carbon employed in a blast furnace for the purpose of generating heat and maintaining the temperature alone, will not be needed for this said heat will be furnished by the current.

In the same way, a lesser quantity of silica will be required owing to the higher temperature of the electric furnace. The exact proportions of carbon and silica as well as 70 of copper and phosphate rock will be readily determined by the skilled furnace man. In the case of a blast furnace it is desirable to use a hot blast, to restrict its amount of air to say 7 pounds to each pound of coke when 75 working with the above mentioned charge, and it is preferred to preheat this said air as high as possible as say up to 1300° F. This enables me to limit the boundaries of the fusion zone, for with a limited quantity 80 of highly heated air the combustion is found not to spread so widely and to be more intense in the fusion zone than is the case when air at a lower temperature and in a greater quantity is employed. The higher 85 temperature is probably due to the preheated air, and the restricted fusion zone is probably due to its limited quantity. The advantage of thus maintaining a very high localized temperature and an excess of carbon 90 in the fusion zone is to deoxidize the evolved  $P_2O_5$  to elemental phosphorus P, as fast as it is formed and thus permit the same to at once enter the reduced or metallic copper present.

95  
Of course, copper oxide or other copper ores can be employed instead of metallic copper in the charge, and when such are used they may be reduced in a manner well known to metallurgists. The conditions being as above outlined and a blast furnace being employed, it will operate with a sufficiently cool top, with a hot bottom, and a localized fusion zone that will not consume 100

too much of the carbon of the charge before the latter reaches the fusion zone in its downward descent, and thus the carbon will be conserved to take care of the reactions 5 which must take place in said fusion zone. The temperatures best suited to the decomposition reactions in said fusion zone range from say 3100° F. down to say 1500° F. At a red heat or at about 1400° F. or 1500° F. 10 the copper begins to absorb the phosphorus vapors and to form cuprous phosphids such as  $Cu_3P$ , and this absorption will continue all the way up to the volatilization point of the copper and even beyond said point. This 15 said compound  $Cu_3P$  dissolves in the copper present, and therefore, it serves to gradually increase the phosphorus content of the whole copper mass in the furnace and this dissolving action continues until a series of 20 solid solutions are formed.

In carrying out this invention, in order to facilitate the permeation of the copper by the free phosphorus, I preferably maintain the partial pressures of the evolved constituents above that of the normal, so that the phosphorus being under an abnormal partial pressure, it will more fully saturate the copper than would otherwise be the case. This said partial pressure may conveniently 25 be made as high as that which would accompany several pounds pressure of the blast above that which is normally employed in pig iron furnaces and is best attained by throttling to a proper degree the down- 30 comer of the furnace. By thus increasing the pressure inside said furnace without increasing the air admitted, and at the same time producing a sufficient quantity of free phosphorus by employing a very high temperature of the blast, a limited quantity of 35 air and thus restricting the fusion zone I am enabled to so thoroughly impregnate the copper present as to produce phosphids of copper of the composition of  $Cu_3P_2$ , and 40 even higher compounds of phosphorus and 45

copper, possibly up to and including the phosphid  $CuP$ .

By carrying out the foregoing process it will now be seen that I am enabled to impregnate copper with any certain, definite 50 percentages of phosphorus from say 4% up to 33%, and that I am thus enabled to supply phosphor-copper compounds for the varied uses now found in the arts, as a product of the blast furnace. On the other 55 hand, when it is desired to produce smaller quantities of said product, I may employ an electric type of furnace. In such latter case in order to reduce the  $P_2O_5$  evolved to elemental phosphorus, I also employ an excess 60 of carbon, but I do not employ any carbon as a source of heat for the heat in such case, as stated above, is furnished by the current. Further when an electric furnace is employed, air is carefully excluded therefrom. 65

What I claim is:—

1. The process of producing phosphor-copper compounds which consists in providing a charge containing copper bearing material, silica, phosphorus bearing material 70 and sufficient carbon to liberate and reduce phosphorus oxids to elemental phosphorus; and heating said charge to a temperature sufficient to cause said elemental phosphorus to impregnate the copper present, substantially as described.

2. The process of producing phosphor-copper compounds in a blast furnace which consists in providing a charge of copper bearing material, silica, phosphate rock, and 80 a sufficient excess of carbon to reduce any evolved phosphorus oxids to elemental phosphorus; admitting air preheated above 1150° F. to said furnace in restricted predetermined quantities; and raising the temperature of said charge material to a point sufficient to cause the reduced phosphorus to enter said copper, substantially as described. 85

In testimony whereof I affix my signature.  
HYLEMAN ALISON WEBSTER.